

# United States Patent

Simon-Vermot

[15] 3,694,885

[45] Oct. 3, 1972

[54] **METHOD OF MANUFACTURING AN  
ESCAPEMENT LEVER FOR A  
TIMEPIECE**

[72] Inventor: **Andre Simon-Vermot, Le Locle,  
Switzerland**

[73] Assignee: **Les Fabriques d'Assortiments Reunies, Le Locle, Neuchatel, Switzerland**

[22] Filed: **July 2, 1970**

[21] Appl. No.: **52,093**

[30] **Foreign Application Priority Data**

July 11, 1969 Switzerland ..... 10607/69

[52] U.S. Cl. .... 29/177, 58/121 R

[51] Int. Cl. .... B23p 13/00

[58] **Field of Search** ... 29/177; 58/116, 121 A, 121 R,  
58/122

3,335,562 8/1967 Schneider ..... 58/122  
3,481,140 12/1969 Tuetey ..... 29/178 X  
3,511,340 5/1970 Simon-Vermot ..... 58/121 A

*Primary Examiner*—John F. Campbell

*Assistant Examiner*—Victor A. Di Palma

*Attorney*—Imirie & Smiley

[57] **ABSTRACT**

A method of manufacturing an escapement lever for a timepiece, characterized by blanking out the lever of a metal sheet, the pallets being made integral with the body of the lever, depositing electroless nickel on to the whole piece and subjecting the lever to a finishing operation carried out so as to obtain cold rolled properties in the layer of chemical nickel, this finishing operation determining the final dimensions of the lever, to which the pallet arbor and the safety-pin are then secured.

[56] **References Cited**

UNITED STATES PATENTS

540,546 6/1895 Hart ..... 29/178

**4 Claims, No Drawings**

## METHOD OF MANUFACTURING AN ESCAPEMENT LEVER FOR A TIMEPIECE

The present invention relates to a method of manufacturing an escapement lever for a timepiece.

The lever of a lever escapement generally consists of a metallic body to which are secured two pallets, usually made of ruby.

Due to its operation, it is difficult to lubricate a lever escapement in a satisfactory manner. Tests have shown that better results can be obtained in this respect by replacing the ruby of the pallets by a body consisting of so-called "electroless nickel", the composition of which is, in fact, an alloy of nickel and phosphorus containing 3.5 to 11.5 percent of phosphorus, the rest being formed by nickel.

Obtaining this alloy by chemical way is relatively long and machining the same to obtain pallets is rather delicate.

The present invention aims at overcoming these drawbacks. It relates to a method of manufacturing an escapement lever for a timepiece, which is broadly characterized by blanking out the lever of a metal sheet, the pallets being made integral with the body of the lever, chemically depositing electroless nickel on to the whole piece, and then subjecting the lever to a finishing operation carried out so as to obtain cold rolled properties in the layer of electroless nickel, this finishing operation determining the final dimensions of the lever, to which the pallet arbor and the safety-pin are then secured.

The metal sheet of which the lever is blanked out may consist, for example, of brass or steel.

The electroless nickel is deposited on the piece by 35 chemical way, by dipping the piece into a suitable bath. The thickness of the coating is preferably less than 50  $\mu$ .

The rolling or laminating effect obtained by the finishing operation guarantees a better adhesion of the coating.

The electroless nickel is not self-lubricating, but has 5 a low coefficient of friction and a high hardness, this representing favorable features. It must be lubricated in order that the escapement operates in a satisfactory manner.

Possibly, the completed lever may be subjected to a 10 heat-treatment at about 800° C so as to increase the hardness of the coating of electroless nickel by precipitation of a phase.

The manufacture of the lever described is easy and inexpensive and the thus obtained lever guarantees a 15 reliable operation and a long working life of the escapement.

What I claim is:

1. A method of manufacturing a timepiece escapement lever including pallets, a pallet arbor and a safety-pin, comprising the steps of: blanking out the lever from a metal sheet, making the pallets integral with the body of the lever, chemically depositing electroless nickel on to the whole piece, subjecting the lever to a fine blanking operation to obtain cold rolled properties 20 in the layer of electroless nickel to determine the final dimensions of the lever, and securing the pallet arbor and the safety-pin to the lever.

2. A method according to claim 1, characterized by 25 depositing the electroless nickel by dipping the piece into a suitable bath.

3. A method according to claim 1, characterized in that the thickness of the coating of electroless nickel is less than 50  $\mu$ .

4. A method according to claim 1, characterized by 30 subjecting the completed lever to a heat-treatment, in order to increase the hardness of the coating of electroless nickel.

\* \* \* \* \*